

April 28, 1936.

E. C. DOMM

2,038,549

METHOD OF COATING METAL

Original Filed Jan. 25, 1933



Inventor:  
Elgin Carleton Domm.  
By Dryerforth, Lee, Clinton & Wills.  
Attest:  
E. C. Domm.

## UNITED STATES PATENT OFFICE

2,038,549

## METHOD OF COATING METAL

Elgin Carleton Domm, Niles, Mich., assignor to  
National-Standard Company, Niles, Mich., a  
corporation of Michigan

Original application January 25, 1933, Serial No.  
653,549. Divided and this application Septem-  
ber 8, 1934, Serial No. 743,282

6 Claims. (Cl. 91—70)

This invention relates to improvements in  
method of coating metal.

In the Crapo Patent No. 1,984,335, issued Dec.  
11, 1934, is described a method of coating a fer-  
rous article by hot-galvanizing it with zinc, and  
over that depositing by some other method an  
additional coating of zinc or a coating of cad-  
mium.

It has now been discovered that a corrosion-  
resisting coating of cadmium may be produced  
which is considerably more resistant to corrosion,  
particularly to the type of which the salt spray is  
typical.

At the same time a relatively thin coating may  
be produced for equivalent protection to such  
corrosion, and such coating may be correspond-  
ingly more exactly controlled as to depth and  
thickness, by the present method.

The invention is particularly applicable to  
coating strands of wire to be used in reinforcing  
the bead of a tire. The wire when so used com-  
monly acts as a tension-member, and is imbedded  
in a rubber or rubber compound. When so used,  
the wire is exposed to corrosive and rusting  
agents, particularly to moisture which may seep  
into the tire.

The drawing shows in diagrammatic form an  
embodiment of my invention.

In accordance with the invention, a metal, for  
example wire suitable for use in tire beads, is first  
hot-dipped to provide a coating of cadmium.  
This may be done, for example, by dipping the  
wire in hot molten cadmium. Another coating  
of cadmium is then put over the first coat by elec-  
trolysis or electroplating.

Not only does a double coating applied by the  
above-mentioned method give very good corrosion  
resistance, but it has been discovered that the  
electro-coat tends to fill in the depressions, in the  
lower cadmium coat and thus produce a uniform  
and smooth coating. This is wholly unexpected.

If desired, copper or other suitable material  
may be applied over the corrosive-resistant coat-  
ing in order to increase the adhesiveness of the  
wire to rubber. It is frequently desirable to  
apply such a coating when wire is used as a rein-  
forcement for a tire bead.

The new process herein described is especially  
useful in procuring a coating of a desired and

uniform thickness. In practice, I give the wire a  
hot coat first, and preferably I have this thin.  
In the next step, when the coating is put on by  
electroplating, the operation can be continued to  
give exactly a desired thickness. At the same 5  
time the coating requires a smooth, uniform  
character which is free from holes, defects, and  
the like.

The foregoing description has been given for  
clearness of understanding only, and no unneces- 10  
sary limitations are to be understood therefrom,  
but the appended claims should be construed as  
broadly as permissible in view of the prior art.

This application is a division of my co-pending  
application Serial Number 653,549, filed January 15  
25, 1933.

What I regard as new and desire to secure by  
Letters Patent is:

1. The process of coating a ferrous article  
which consists in applying to it by the hot-dip 20  
process a coating of cadmium, and electrode-  
depositing thereon an outer coating substantially  
wholly of cadmium.

2. The method of coating a metal to increase  
its corrosion resistance comprising first applying 25  
to it molten cadmium, and then applying a sec-  
ond coating of cadmium by electroplating over  
the first coating.

3. The method of producing a ferrous tire-  
bead reinforcement wire of uniform corrosion- 30  
resistance which comprises first coating a ferrous  
wire with cadmium by the hot-dip process, and  
then electroplating cadmium upon the hot-dip  
wire to produce a uniform coating of desired  
thickness. 35

4. A coated ferrous article, comprising a fer-  
rous base having a hot-dipped coating of cad-  
mium thereon, and over that an electrodeposited  
coating substantially wholly of cadmium.

5. A coated ferrous wire, comprising a ferrous 40  
base wire having a hot-dipped coating of cad-  
mium thereon, and over that an electrodeposited  
coating substantially wholly of cadmium.

6. A coated tire bead wire comprising a ferrous 45  
base wire having a hot-dipped coating of cad-  
mium thereon, an electrodeposited coating sub-  
stantially wholly of cadmium thereon, and having  
a coating of rubber vulcanized thereto.

ELGIN CARLETON DOMM.

50